

# United States Patent [19]

Ferguson

[11] 3,900,321

[45] Aug. 19, 1975

[54] SILVER HALIDE EMULSION CONTAINING  
AROMATIC AZOCARBONAMIDE ANTIFOG  
AGENT

[75] Inventor: Alan Norman Ferguson, Harlow,  
England

[73] Assignee: Minnesota Mining and  
Manufacturing Company, St. Paul,  
Minn.

[22] Filed: Oct. 2, 1972

[21] Appl. No.: 293,772

[30] Foreign Application Priority Data

Oct. 18, 1971 United Kingdom..... 47056/71

[52] U.S. Cl..... 96/76 R; 96/109; 260/192;  
260/553; 96/66.5

[51] Int. Cl. .... G03c 1/48; G03c 1/34

[58] Field of Search..... 96/109, 66.5, 76 R;  
260/192, 553

[56] References Cited  
UNITED STATES PATENTS

3,655,391 4/1972 Merli et al. .... 96/109  
3,732,104 5/1973 Vandenabeele et al. .... 96/109

Primary Examiner—Won H. Louie, Jr.  
Attorney, Agent, or Firm—Alexander, Sell, Steldt &  
DeLaHunt

[57] ABSTRACT

Aromatic azocarbonamides act as antifogging agents when included in silver halide photographic emulsions without seriously affecting film speed, contrast or maximum densities.

10 Claims, No Drawings

SILVER HALIDE EMULSION CONTAINING  
AROMATIC AZOCARBONAMIDE ANTIFOG  
AGENT

This invention relates to photographic silver halide emulsions containing organic anti-fogging agents and

It is believed that these azocarbonamides act as anti-fogging agents for photographic emulsions because they can be readily reduced, i.e., they are oxidizing agents, and they oxidize developable silver halide specks to a non-developable form. This oxidation is illustrated for example, by the following reaction using phenylazocarbonamide:



to ring-substituted azocarbonamides for use as anti-fogging agents for photographic silver halide emulsions.

According to the invention there is provided a photographic silver halide emulsion which has in fog inhibiting reactive association therewith an azocarbonamide.

We find that these azocarbonamides act as anti-fogging agents for photographic emulsions. It is believed that the desired anti-fogging effect is achieved because the azocarbonamide acts as an oxidizing agent for those silver halide crystals or grains in the emulsion which become accidentally developable, i.e., fogged, during production or handling of the emulsion, e.g., by accidental slight light exposure, chemical action or strain. Thus when a crystal or grain becomes fogged, it is oxidized by the azocarbonamide and so the crystal or grain does not therefore become developed as a fog speck when the emulsion is developed after normal light exposure.

The azocarbonamide is preferably added to the photographic emulsion. It can instead be present in a layer adjacent to an emulsion layer.

The optimum amount of azocarbonamide to be added to a photographic emulsion to give the desired anti-fogging effect can easily be found by simple experiment. In general, however, good results will be given when from 0.025 to 1.0 millimole of an azocarbonamide, and preferably a ring-substituted azocarbonamide, is added per mole of silver in the emulsion. When added in these amounts, the azocarbonamide does not seriously effect the other desirable properties of the emulsion such as film speed, and in addition we find that the azocarbonamide has comparable or better anti-fogging properties and also comparable or better gamma (contrast) and D-max when added to photographic emulsions as compared with azodicarbonamide. Also it is often possible to add less of the azocarbonamide, and particularly a ring-substituted azocarbonamide, than azodicarbonamide to achieve comparable anti-fogging properties.

Certain of the azocarbonamides of this invention, and particularly ring-substituted azocarbonamides, are 30 unstable when in contact with the emulsion, e.g., hydrolytically unstable, and are decomposable in a reasonable time at normal temperatures, e.g., 60 days at 60°F, to innocuous decomposition products. Therefore these azocarbonamides can be added to photographic 35 silver halide emulsions in relatively large amounts, i.e., in an amount which is at least sufficient to oxidize the silver in those silver halide crystals or grains which would otherwise become developable after the emulsion has been prepared and coated on a suitable substrate and dried, any excess azocarbonamide being capable of decomposing in a reasonable time at normal 40 temperatures to leave insufficient azocarbonamide to interfere substantially with image exposure and development of the emulsion coating.

Therefore certain azocarbonamides and preferably 45 ring-substituted azocarbonamides can be used as the oxidizing agent required to eliminate undesirable fog in photographic elements according to the inventions described in our copending U.S. patent application Ser. 50 Nos. 243,463 and 244,276, filed Apr. 12, 1972 and Apr. 14, 1972 respectively. They are added to the emulsion in relatively large amounts, e.g., from 1.5 to 25 millimoles per mole of silver in the emulsion and initially they almost completely desensitize the emulsion 55 to light. However, they decompose in a reasonable time so that they protect the emulsion from fog formation during manufacture and coating of the emulsion and handling of the coated emulsion, and then the emulsion regains its speed before use.

The photographic emulsion to which the azocarbonamides can be added can be one which is suitable for 60 black and white or for color photography, or for use in radiography. Also the emulsion can be a negative emulsion or a direct positive emulsion. Further the silver halide can be the bromide, iodide, a mixed halide or any of the silver halide materials useful in photographic 65 techniques.

The preferred azocarbonamides used in photographic emulsion according to the invention are aryl azocarbonamides, preferably ring-substituted azocarbonamides represented by the formula:



wherein Ar represents any aromatic group and R represents a carbonamide. According to one aspect of the invention there is provided an novel azocarbonamide represented by the formula:



wherein Ar represents any aromatic group and R represents a carbonamide with the exception of the case where both Ar represents a phenyl group and R represents the group  $-\text{CONH}_2$ . The preferred carbonamide groups may be further characterized as



in which  $\text{R}^1$  and  $\text{R}^2$ , which may be the same or different, each represents a hydrogen atom, an alkyl, alkylene, alicyclic, aryl, aralkyl, alkaryl group or a grouping containing a center of positive charge and having associated with it one or more negatively charged moieties sufficient to impart electrical neutrality, or  $\text{R}^1$  and  $\text{R}^2$  together with the nitrogen atom to which they are linked represent the atoms required to complete a heterocyclic ring which may itself be substituted or contain a center of positive charge having associated with it one or more negatively charged moieties sufficient to impart electrical neutrality, with the exception of the case where Ar represents a phenyl group and  $\text{R}^1$  and  $\text{R}^2$  both represent hydrogen atoms. Those compounds which are suitable for use according to the invention described in our above noted copending U.S. patent applications oxidizing agents having an oxidizing potential of from  $-0.08$  to  $+0.50$ . These compounds are hydrolytically unstable in that they decompose when in contact with an emulsion within about 60 days at  $60^\circ\text{F}$ .

Illustrative of the types of groups which can be used for the aromatic group Ar are, for example, an aryl, aralkyl or alkaryl group such as a phenyl, naphthyl, or substituted phenyl group of the general formula:



or substituted naphthyl group of the general formula:



or a heterocyclic group which can contain a quaternizable nitrogen atom such as one of the groups having the general formula:



in which the groupings represented by  $\text{R}^3$  may be different from one another and are a hydrogen or halogen atom or an alkyl, alkylene, alicyclic, aryl, aralkyl, alkaryl,  $-\text{COOH}$ ,  $-\text{SO}_3\text{H}$ , alkyl ammonium or fluoroalkyl group.

The most preferred class of azocarbonamides which ace particularly well as excellent anti-fogging agents are those where Ar represents a phenyl or a naphthyl group. These may be substituted phenyl or naphthyl groups as well as unsubstituted. Also heterocyclic groups as set out above and  $\text{R}^1$  and  $\text{R}^2$  represent hydrogen atoms or lower alkyl groups, e.g., containing 1 to 4 carbon atoms may be used. In order to improve the water solubility of such compounds the grouping Ar may contain one or more water-solubilizing groups such as  $-\text{COOH}$  or  $-\text{SO}_3\text{H}$ . Substituents such as  $-\text{NO}_2$  tend to desensitize photographic emulsions and so are preferably not present.

These azocarbonamides are relatively hydrolytically stable and so will generally be added in quite small amounts as noted above to photographic emulsions to act as anti-fogging agents. Generally the water solubility of these compounds is sufficient to enable them to be added in these relatively small amounts in aqueous solution which has the advantage of being compatible with the emulsion and relatively inert to the emulsion.

When the azocarbonamides contain groupings having centers of positive charge, e.g., quaternary ammonium groupings, they can have the general formula:



or more particularly



in which R represents a carbonamide wherein a substituent in the nitrogen atom of the carbonamide group contains at least one quaternary ammonium,  $\text{R}^1$  represents a grouping containing at least one quaternary ammonium grouping,  $\text{R}^2$  represents a hydrogen atom or an aliphatic, alicyclic, aromatic or heterocyclic group, or  $\text{R}^1$  and  $\text{R}^2$  together with the amide nitrogen atom com-

plete a 5 or 6 membered heterocyclic ring, which may be substituted, and which contains either in the ring or on a substituent group one or more nitrogen atoms which are the centers of positive charge, X represents one or more negatively charged ions sufficient to give the azocarbonamide electrical neutrality, and Ar represents an aromatic grouping as defined above.

Illustrative of a suitable grouping to be represented by R<sup>1</sup> is



while an example of a suitable grouping represented by R<sup>1</sup> and R<sup>2</sup> together with the amide nitrogen is



where R<sup>4</sup> represents a lower alkyl group.

The negatively charged moiety or moieties can be one or more separate anions associated with the azocarbonamide or the azocarbonamide can also contain one or more negatively charged substituents as part of its structure. In the case where the azocarbonamide has associated with it one or more separate anions, suitable anions include, for example, aryl sulphonates such as toluene-p-sulphonate, alkyl sulphites, boron tetrafluoride (BF<sub>4</sub><sup>-</sup>), iodide, iodate, chloride, chlorate, perchlorate and nitrate ions. On the other hand where the negatively charged moiety forms part of the azocarbonamide, the negatively charged grouping can include, for example, a sulphobetain grouping.

These charged azocarbonamides are readily soluble in water and so they can readily be incorporated into photographic emulsions without the use of organic solvents which, besides being expensive, may have undesirable side effects upon the emulsion. Also their good solubility enables them to be distributed throughout the emulsion very uniformly. Further their ready water solubility enables one to incorporate relatively large amounts of them into the emulsion as required according to our copending U.S. patent application Ser. Nos. 243,463 and 244,276.

Many of the ring-substituted azocarbonamides of the invention can be prepared by oxidizing (e.g., with acidified potassium permanganate), the corresponding ring-substituted hydrazocarbonamide. Depending upon the particular ring-substituted azocarbonamide, this intermediate hydrazocarbonamide can be prepared in a number of ways.

Thus a phenylazocarbonamide, substituted or unsubstituted on the phenyl ring and unsubstituted on the amide nitrogen atom, can be prepared by reacting the corresponding phenylhydrazine, preferably as its hydrochloride salt, with a cyanate, e.g., KCNO, and then oxidizing the resulting phenyl hydrazocarbonamide. This reaction is illustrated by the following scheme for preparing N-p-ethylphenylazocarbonamide:



15

A phenylazocarbonamide substituted or unsubstituted on the phenyl ring and mono- substituted on the amide nitrogen atom can be prepared by reacting the corresponding phenylhydrazine with the appropriate isocyanate followed by oxidation of this intermediate hydrazocarbonamide. This reaction is illustrated by the following scheme for preparing N-ethylphenylazocarbonamide:



40

A phenylazocarbonamide substituted or unsubstituted on the phenyl ring and di-substituted on the amide nitrogen atom can be prepared by reacting the corresponding phenylhydrazine with the appropriate di-substituted carbamyl chloride, e.g., a dialkyl chloride, followed by oxidation of the resulting intermediate hydrazocarbonamide. This reaction is illustrated by the following scheme for preparing N-dimethylphenylazocarbonamide:



60

A heterocyclic azocarbonamide unsubstituted on the amide nitrogen atom can be prepared by reacting the corresponding heterocyclic hydrazine, preferably in the form of a salt with a cyanate, e.g., KCNO, and then oxidizing the resulting heterocyclic hydrazocarbonamide. This reaction can be illustrated by the following scheme for preparing 2-quinolineazocarbonamide:



Another route for the preparation of the ring-substituted azocarbonamides is to react the corresponding azo ester with a diamine. This route is particularly useful for the preparation of azocarbonamides which have tertiary amine substituents.

Thus a heterocyclic azocarbonamide which is mono- or di- substituted on the amide nitrogen atom can, for example, be prepared by making the corresponding heterocyclic hydrazone, oxidizing this to the azo ester followed by reaction with a diamine. This diamine may form with the azo ester an azocarbonamide in which the amine nitrogen atom forms part of a heterocyclic ring containing a second tertiary nitrogen atom or an azocarbonamide in which one substituent on the amine nitrogen atom contains a tertiary nitrogen atom. The following reaction scheme illustrates this procedure:

Azocarbonamides containing a quaternary ammonium group can be prepared from azocarbonamides substituted on the amide nitrogen atom with a grouping containing a tertiary nitrogen atom by reacting with a quaternizing agent such as p-toluene sulphonate or ethyl iodide.

The invention will now be illustrated, by way of example, with reference to the following preparation of phenylazocarbonamide, Examples 1 to 33 illustrating the preparation of other azocarbonamides, and Examples 34 to 36 illustrating the use of azocarbonamides in photographic silver halide emulsions.

## PREPARATION

### Phenylazocarbonamide

Potassium cyanate (16.2 g, 0.2M) in water (50 ml)

30



Also phenylazocarbonamides substituted or unsubstituted on the phenyl ring and mono- or di- substituted on the amide nitrogen atom in which one or both substituents on the amide nitrogen atom contain a tertiary nitrogen atom or the amide nitrogen atom forms part of a heterocyclic ring containing a second tertiary nitrogen atom can be made in a similar fashion to the above heterocyclic azocarbonamides. This can be illustrated by the following reaction scheme:

50 was added with stirring to a solution of phenylhydrazine hydrochloride (29.0 g, 0.2 M) in water (100 ml) at room temperature. Almost immediately a heavy white precipitate of 1-phenylsemicarbazide came down. The precipitate was filtered off, washed with a little cold water and dried.

55 A solution of potassium permanganate (7.0 g), dilute sulphuric acid (45 ml, 1N) and water (150 ml) was heated to 70°C and slowly added with stirring to a solu-



tion of 1-phenylsemicarbazide (10.0 g, 0.066 M) in water (200 ml), at 80°C.

The hot solution was then filtered. On cooling phenylazocarbonamide crystallized out as golden plates. The product was filtered off and dried under vacuum. The yield was 7.0 g (melting point 114°C).

A sample for analysis was recrystallized from carbon tetrachloride.

Analysis:  $C_7H_7N_3O$  requires: C 56.4%; H 4.7%; N 28.2%; found: C 56.1%; H 4.6%; N 27.7%.

#### EXAMPLE 1

##### N-Ethylphenylazocarbonamide

Phenylhydrazine (21.6 g, 0.2M) was dissolved in benzene (25 ml) and added dropwise, with stirring, to a solution of ethylisocyanate (14.3 g, 0.2M) in benzene (25 ml). After addition was complete the reaction mixture was refluxed for ½ hour. On cooling, a white crystalline precipitate of the 1-phenyl-4-ethyl semicarbazide was formed. Filtering, washing with cold water and vacuum drying gave 30 g of the intermediate.

1-Phenyl-4-ethylsemicarbazide (11.8 g, 0.066M) was oxidized as described in the preparation to give a yellow crystalline solid which was recrystallized from cyclohexane/ethyl acetate mixture to give 5.2 g of the desired product (melting point 55°–56°C).

Analysis:  $C_9H_{11}N_3O$  requires: C 61.1%; H 6.2%; N 23.8%; found: C 61.1%; H 6.2%; N 23.1%.

#### EXAMPLE 2

##### N-Dimethylphenylazocarbonamide

Dimethylcarbonylchloride (21.5 g, 0.2M) was added slowly with stirring to an ice-cooled solution of phenylhydrazine (21.6 g, 0.2M) in pyridine (125 ml). After addition was complete, stirring was continued for 2 hours at 20°C. The reaction mixture was then poured into 500 ml. of ice-water. The cream colored solid precipitate was filtered off, washed with cold water and dried at 60°C. The yield of 4,4-dimethyl-1-phenylsemicarbazide was 12.3 g (melting point 160°C).

4,4-Dimethylsemicarbazide (11.8 g, 0.066M) was dissolved in 600 ml of water at 80°C and oxidized as described in the preparation to give an orange solid product which was recrystallized from ethanol. The yield was 3.0 g (melting point 73°C).

Analysis:  $C_9H_{11}N_3O$  requires: C 61.0%; H 6.2%; N 23.75%; found: C 61.4%; H 6.0%; N 24.0%.

#### EXAMPLE 3

##### p-Fluorophenylazocarbonamide

Potassium cyanate (12.6 g, 0.155M) in water (50 ml) was added with stirring to a solution of 4-fluorophenylhydrazine hydrochloride (25.0 g, 0.154M) in water (300 ml) at room temperature. The heavy precipitate of 1-(p-fluorophenyl)semicarbazide which quickly came down was filtered off, washed with cold water and vacuum dried. The yield was 30.0 g (melting point 202°–203°C).

1-(p-Fluorophenyl)semicarbazide (11.2 g, 0.066M) was dissolved in 350 ml of boiling water and oxidized as described in the preparation, to give a yellow solid product which was recrystallized from benzene. The yield was 6.7 g (melting point 138°C).

Analysis:  $C_7H_6N_3OF$  requires: C 50.3%; H 3.6%; N 25.2%; found: C 50.4%; H 3.6%; N 24.7%.

#### EXAMPLE 4

##### o-Tolylazocarbonamide

Potassium cyanate (13.0 g, 0.158M) in water (50 ml) was added with stirring to a solution of o-tolylhydrazine hydrochloride (25.0 g, 0.158M) in water (200 ml) at room temperature. The heavy white precipitate of 1(o-tolyl)semicarbazide which quickly came down was filtered off, washed with cold water and vacuum dried. The yield was 27.5 g (melting point 163°–4°C).

1-(o-Tolyl)semicarbazide (11.0 g, 0.066M) was dissolved in 200 ml of boiling water and oxidized as described in the preparation, to give a pale yellow solid which was recrystallized from benzene to give 9.2 g of yellow crystals (melting point 115°C).

Analysis:  $C_8H_9N_3O$  requires: C 58.9%; H 5.5%; N 25.8% found: C 59.1%; H 5.3%; N 25.4%.

#### EXAMPLE 5

##### 2-Quinolylazo[N-(4-methyl piperazine)amide]

Ethylcarbazate (16.6 g, 0.16M) in ethanol (30 ml) was added to a solution of 2-chloroquinoline (26.0 g, 0.16M) in ethanol (70 ml) containing concentrated hydrochloric acid (10 ml). The reaction mixture was then refluxed for 3 hours, cooled and neutralized with dilute ammonia solution. The white solid precipitate formed was filtered off and recrystallized from ethanol to give 23.5 g of white crystals of ethyl-2-quinolylhydrazocarboxylate (melting point 167°–8°C).

1-Chlorobenzotriazole (7.83 g, 0.05M) was dissolved in methylene dichloride (75 ml) and added dropwise to a stirred solution of ethyl-2-quinolylhydrazocarboxylate (11.6 g, 0.05M) in methylene dichloride (150 ml). Ice cooling was used to keep the temperature below 20°C during the addition. The reaction mixture was then stirred for 1 hour at room temperature, filtered and the filtrate washed with 2 Normal NaOH (25 ml), then water (25 ml) and finally dried over sodium sulphate. Evaporation of the methylene dichloride gave ethyl-2-quinolylazocarboxylate as a dark orange solid (melting point 57°C).

Ethyl-2-quinolylazocarboxylate (4.6 g, 0.02M) was dissolved in ether (50 ml) and stirred while N-methyl-piperazine (2.2 g, 0.022M) was slowly added. The reaction mixture was stirred over-night at room temperature then the precipitate formed was filtered off and recrystallized from cyclohexane to give 4.0 g of orange-red needles of 2-quinolylazo[N-(4-methylpiperazine)amide] (melting point 118°C).

Analysis:  $C_{15}H_{17}N_5O$  requires: C 63.6%; H 6.0%; N 24.8% found: C 63.3%; H 6.0%; N 24.7%.

#### EXAMPLE 6

##### 2-Quinolylazocarbon-(N-piperidino)amide

Piperidine (2.12 g, 0.025M) in ether (20 ml) was added dropwise to a stirred solution of ethyl-2-quinolylazocarboxylate (5.7 g, 0.025M) in ether (200 ml). The reaction was stirred for 1 hour at room temperature and the orange solid precipitate was filtered off. Recrystallization from 80°–100° petroleum ether gave 4.3 g of an orange solid (melting point 127°–8°C).

Analysis:  $C_{15}H_{16}N_4O$  requires: C 67.2%; H 6.0%; N 20.9% found: C 67.0%; H 5.9%; N 20.9%.

## EXAMPLE 7

p-nitro-phenylazocarbon(N-(4-ethyl-4-methyl-piperazinium))amide iodide

Example 7 and quaternizing the appropriate azodicarbonamide having a tertiary amino substituent with the appropriate quaternizing agent as shown in the following Table I.

Table I

| Example No. | Formula | Solvent for recrystallization | Analysis (%)                                                                                                     |
|-------------|---------|-------------------------------|------------------------------------------------------------------------------------------------------------------|
| 8           |         | not recrystallized            | $C_{21}H_{21}N_5O_6S$ requires<br>C 53.5; H 4.5;<br>N 14.9; S 6.8;<br>found:<br>C 52.0; H 4.4;<br>N 12.2; S 7.3; |
| 9           |         | ethanol                       | $C_{17}H_{22}N_5OI$ requires<br>C 46.5; H 5.0;<br>N 16.0; I 29.0;<br>found:<br>C 46.1; H 5.0;<br>N 15.8; I 28.5; |

p-nitro-phenylazocarbon N-(4-methylpiperazine)-amide (2.0 g) was dissolved in ethyl iodide (20 ml) at room temperature and allowed to stand overnight. The orange-yellow solid product was filtered off, washed with ether and dried under vacuum. The yield was 2.3 g.

Structural formula:



Analysis:  $C_{14}H_{20}N_5O_3I$  requires: C 38.8%; H 4.6%; N 16.2%; found: C 38.9%; H 4.5%; N 15.4%.

## EXAMPLES 8 and 9

Other azocarbonamides containing centers of positive charge were prepared following the procedure of

## EXAMPLES 10 to 18

30 The following general reaction was used.  
30 Potassium cyanate (16.2 g; 0.2 M) in water (50 ml) was added with stirring to a solution of the arylhydrazine hydrochloride (0.2 M) in water (100 ml) at room temperature. Almost immediately, a heavy white precipitate of 1-arylsemicarbazide came down. The precipitate was filtered off, washed with a little cold water and dried.

35 A solution of potassium permanganate (7.0 g), dilute sulphuric acid (45 ml, 1 N) and water (50 ml) was heated to 70°C and slowly added, with stirring, to a solution of the 1-arylsemicarbazide (0.066 M) in water (200 ml) at 80°C. The hot solution was then filtered. The arylazocarbonamide which crystallized on cooling was filtered off and dried under vacuum. Recrystallization gave pure products.

40 45 The compounds prepared and their properties are listed in the following Table II.

Table II

| Example No. |  | Melting point (°C) | Solvent for recrystallization | Analysis (%)                                                                                 |
|-------------|--|--------------------|-------------------------------|----------------------------------------------------------------------------------------------|
| 10          |  | 142                | water                         | $C_9H_9N_3O$ requires:<br>C 58.9; H 5.5;<br>N 25.8;<br>found:<br>C 58.8; H 5.3;<br>N 25.4;   |
| 11          |  | 137-8              | benzene                       | $C_7H_7N_3OCl$ requires:<br>C 45.8; H 3.3;<br>N 22.9;<br>found:<br>C 45.6; H 3.4;<br>N 22.3; |

Table II-Continued

| Example No. | N—NCONH <sub>2</sub>                                                              | Melting point (°C) | Solvent for recrystallization | Analysis (%)                                                                                                          |
|-------------|-----------------------------------------------------------------------------------|--------------------|-------------------------------|-----------------------------------------------------------------------------------------------------------------------|
| 12          |  | 121                | ethanol/water 1:10            | C <sub>7</sub> H <sub>6</sub> N <sub>3</sub> OCl<br>requires: C 45.8; H 3.3; N 22.9;<br>found: C 44.6; H 3.2; N 22.3; |
| 13          | R = 4—Cl<br>R' = H                                                                | 188                | benzene                       | C <sub>7</sub> H <sub>6</sub> N <sub>3</sub> OCl<br>requires: C 45.8; H 3.3; N 22.9;<br>found: C 45.8; H 3.4; N 22.3; |
| 14          | R = 2—Cl<br>R' = 6—Cl                                                             | 161                | ethanol/water 1:10            | C <sub>7</sub> H <sub>6</sub> N <sub>3</sub> OCl<br>requires: C 38.6; H 2.3; N 19.3;<br>found: C 38.0; H 2.4; N 18.9; |
| 15          | R = 3—Br<br>R' = H                                                                | 138                | ethanol/water 1:5             | C <sub>7</sub> H <sub>6</sub> N <sub>3</sub> OBr<br>requires: C 36.9; H 2.6; N 18.4;<br>found: C 36.6; H 2.6; N 17.9; |
| 16          | R = 2—F<br>R' = H                                                                 | 131                | ethanol/water 1:1             | C <sub>7</sub> H <sub>6</sub> N <sub>3</sub> OF<br>requires: C 50.3; H 3.6; N 25.2;<br>found: C 50.3; H 3.6; N 25.1;  |
| 17          | R = 3—F<br>R' = H                                                                 | 112                | ethanol/water 1:5             | C <sub>7</sub> H <sub>6</sub> N <sub>3</sub> OF<br>requires: C 50.3; H 3.6; N 25.2;<br>found: C 50.1; H 3.6; N 24.9;  |
| 18          | R = 4—COOH<br>R' = H                                                              | 205                | acetic acid                   | C <sub>8</sub> H <sub>7</sub> N <sub>3</sub> O<br>requires: C 49.8; H 3.6; N 21.8;<br>found: C 48.6; H 3.9; N 20.0;   |

## EXAMPLE 19

## p-Sulphophenylazocarbonamide

p-Sulphophenylhydrazine (37.6 g; 0.2 M) was suspended in water (150 ml) and stirred while a solution of potassium cyanate (16.2 g; 0.2 M) in water (50 ml) was added. The reaction warmed spontaneously and a clear solution was obtained. After 1 hour concentrated hydrochloric acid was added until no further precipitation occurred then stirring was continued for a further 1 hour. The white solid product was filtered off and dried under vacuum over KOH pellets.

The yield was 39.5 g.

1-p-Sulphophenylsemicarbazide (11.5 g; 0.05 M) from the above reaction was suspended in acetonitrile (300 ml) and stirred while 1-chlorobenzotriazole (15.4 g; 0.10 M) in acetonitrile (150 ml) was added dropwise. An orange color developed in the reaction mix-

ture during the addition. When addition was complete stirring was continued overnight at room temperature then the orange solid formed was filtered off, washed with acetonitrile and dried under vacuum.

The yield was 18.0 g.

The product was purified by recrystallization from glacial acetic acid and was shown by elemental analysis to be the benzotriazole salt of p-sulphophenylazocarbonamide.

Analysis: C<sub>13</sub>H<sub>12</sub>N<sub>6</sub>O<sub>4</sub>S requires: C 44.8%; H 3.5%; N 24.1%; found: C 44.8%; H 3.7%; N 23.2%.

## EXAMPLES 20 to 23

Phenylsemicarbazide substituted or unsubstituted on the phenyl ring and mono-substituted on the amide nitrogen can be prepared by reaction of the appropriate phenylhydrazine with an isocyanate followed by oxida-



To a solution of the above hydrazo compound (22.5 g; 0.10 M) in methylene dichloride (100 ml) was added dropwise, with stirring, a solution of 1-chlorobenzotriazole (15.4 g; 0.10 M) in methylene dichloride (50 ml). The reaction mixture was stirred for 1 hour at room temperature and the benzotriazole hydrochloride formed was filtered off. The filtrate was evaporated to give 18.6 g of ethyl-p-nitrophenylazocarboxylate as a golden brown solid.

The azocarboxylate (8.8 g; 0.04 M) was dissolved in ether (50 ml) and stirred while a solution of 4-aminomethylpyridine (4.4 g; 0.04 M) in ether (15 ml) was run in slowly. An orange-red precipitate was quickly formed. Stirring was continued for 1 hour, then the product was filtered off and recrystallized from acetone to give 9.3 g of orange platelets.

Other analogous azocarbonamides were prepared in a similar fashion and their properties are listed in the following Table IV.

Table IV

| Example No. |  | Melting point (°C) | Solvent for recrystallization | Analysis (%)                                                                                                                                   |
|-------------|-----------------------------------------------------------------------------------|--------------------|-------------------------------|------------------------------------------------------------------------------------------------------------------------------------------------|
| 26          | R=R'=R''=H<br>R'''=3—CH <sub>2</sub> —<br>Pyridyl                                 | 120                | ethanol                       | C <sub>13</sub> H <sub>12</sub> N <sub>4</sub> O<br>requires:<br>C 65.0; H 5.0;<br>N 23.4;<br>found:<br>C 65.5; H 5.6;<br>N 23.5;              |
| 27          | R=4—NO <sub>2</sub> R'=R''=H<br>R'''=3—CH <sub>2</sub> —<br>Pyridyl               | 180                | acetonitrile                  | C <sub>13</sub> H <sub>11</sub> N <sub>5</sub> O <sub>3</sub><br>requires:<br>C 54.7; H 3.9;<br>N 24.6;<br>found:<br>C 54.8; H 4.0;<br>N 24.4; |
| 28          | R=4NO <sub>2</sub> R'=R''=H<br>R'''=2—CH <sub>2</sub> —<br>Pyridyl                | 136                | acetonitrile                  | C <sub>13</sub> H <sub>11</sub> N <sub>5</sub> O <sub>3</sub><br>requires:<br>C 54.7; H 3.9;<br>N 24.6<br>found:<br>C 55.1; H 4.3;<br>N 24.5;  |
| 29          | R=4—NO <sub>2</sub> R'=R''=H<br>R'''=4CH <sub>2</sub> —<br>Pyridyl                | 172                | acetonitrile                  | C <sub>13</sub> H <sub>11</sub> N <sub>5</sub> O <sub>3</sub><br>requires:<br>C 54.7; H 3.9;<br>N 24.6;<br>found:<br>C 54.9; H 3.8;<br>N 24.6. |

## EXAMPLE 30

## 2-Quinolineazocarbonamide

2-Hydrazinoquinoline (23.85 g, 0.15 M) was stirred in water (100 ml) and concentrated hydrochloric acid (5.5 g, 0.15 M) was added. To this solution was added, with stirring, a solution of potassium cyanate (12.15 g, 0.15 M) in water (25 ml). A white solid precipitate of the quinoline-hydrazocarbonamide formed and was filtered off, washed with a little water and dried in vacuum.

The yield was 23.0 g.

The crude quinolinehydrazocarbonamide (20.2 g, 0.10 M) was dissolved/suspended in methylene dichlo-

ride and stirred while a solution of 1-chlorobenzotriazole (15.4 g, 0.10 M) in methylene dichloride (100 ml) was added dropwise. External ice-cooling was used to keep the temperature below 20°C during the addition. After addition was complete, a further 2 hours stirring at room temperature was given, then the reaction mixture was filtered.

The filtrate was washed with 2 Normal NaOH (50 ml), followed by water (50 ml) and dried over Na<sub>2</sub>SO<sub>4</sub>. Evaporation of the filtrate gave 5.2 g of an orange-red solid which was recrystallized from ethanol (melting point 161°-2°C).

Analysis: C<sub>10</sub>H<sub>8</sub>N<sub>4</sub>O requires: C 60.0%; H 4.0%; N 28.0%; found: C 60.0%; H 4.0%; N 27.7%.

## EXAMPLE 31

A coarse-grain gelatine silver bromoiodide emulsion, of cubic habit and having a mean grain size of approximately 2.0 microns, was prepared by ripening under

15

ammoniacal conditions, the final emulsion having an iodide content of about 2 moles percent. The emulsion was digested with a sulphur and a gold sensitizer. After stabilization by the addition of 4-hydroxy-5-2-hydroxyethyl-6-methyl-1:3:3a:7-tetraazaindene 3-amino-5-methylthio-1:2:4-triazole salt (see Example 1 of our United Kingdom Pat. No. 1,022,872), the emulsion was divided into four parts. To one part (Emulsion A) no addition was made while to the second part (Emulsion B) an aqueous solution of azodicarbonamide was added, to the third part (Emulsion C) an aqueous solution of m-bromo-phenylazocarbonamide was added, and to the fourth part (Emulsion D) an aqueous solution of m-chlorophenylazocarbonamide.

55 ammoniacal conditions, the final emulsion having an iodide content of about 2 moles percent. The emulsion was digested with a sulphur and a gold sensitizer. After stabilization by the addition of 4-hydroxy-5-2-hydroxyethyl-6-methyl-1:3:3a:7-tetraazaindene 3-amino-5-methylthio-1:2:4-triazole salt (see Example 1 of our United Kingdom Pat. No. 1,022,872), the emulsion was divided into four parts. To one part (Emulsion A) no addition was made while to the second part (Emulsion B) an aqueous solution of azodicarbonamide was added, to the third part (Emulsion C) an aqueous solution of m-bromo-phenylazocarbonamide was added, and to the fourth part (Emulsion D) an aqueous solution of m-chlorophenylazocarbonamide.

65

was added. After the addition of necessary coating aids, the emulsions were coated on polyester bases to give a silver coating weight of 5.0 g/meter<sup>2</sup>. Each emulsion layer was then coated with a protective gelatin super coat containing a gelatin cross-linking agent. The coated films were dried, exposed to a continuous wedge in a sensitometer, and processed at 104°F in a standard, commercially-available developer of the type suitable for use in a modern X-ray film processing machine having a total dry-to-dry process time of 90 seconds. The relative fog speeds, fog levels, gamma and D-max were measured and results were as shown in the following Table V.

Table V

| Emul-sion | Amount of anti-fogging agent added, M/40 aqueous solution (ml) | Fog  | Relative log speed |      | D-max |
|-----------|----------------------------------------------------------------|------|--------------------|------|-------|
|           |                                                                |      | amma               | amma |       |
| A         | —                                                              | 0.07 | 1.65               | 1.56 | 1.87  |
| B         | 25                                                             | 0.05 | 1.65               | 1.62 | 1.85  |
| C         | 1                                                              | 0.05 | 1.70               | 1.59 | 1.92  |
| D         | 3                                                              | 0.04 | 1.68               | 1.59 | 1.83  |

The amounts of the aqueous solutions added in each case was the optimum amount.

As can be seen from these results, the anti-fogging effects of the ring-substituted azocarbonamides in the emulsions according to the invention (Emulsions C and D) were excellent as compared with the Emulsion A without any addition, and also as good as or better than the anti-fogging effects of azodicarbonamide (Emulsion B), even though much smaller amounts of the ring-substituted azocarbonamides were added to Emulsions C and D. It will further be noted that the other photographic properties of the emulsions according to the invention were similar to the emulsion without addition (Emulsion A).

## EXAMPLE 32

Coarse-grain gelatine or silver bromoiodide emulsions, of cubic habit and having a mean grain size of approximately 2.0 microns, were prepared by ripening under ammoniacal conditions, the final emulsions having iodide contents of about 2 moles percent. The emulsions were digested with a sulphur and gold sensitizer. After stabilization by the addition of 4-hydroxy-5-2-hydroxyethyl-6-methyl-1:3:3a:7-tetraazaindene 3-amino-5-methylthio-1:2:4-triazole salt, additions of aqueous solutions of various azocarbonamides in various amounts (ml of azocarbonamide per mole of silver in the emulsion) were made as shown in the following Tables VI to X for comparison purposes, no addition and the addition of an aqueous solution of azodicarbonamide were also made.

After the addition of the necessary coating aids, the emulsions were coated on polyester bases to give a silver coating weight of 5.0 g/meter<sup>2</sup>. Each emulsion layer was then coated with a protective gelatin super coat containing a gelatin cross-linking agent. The coated films were then dried, exposed to a continuous wedge in a sensitometer and processed at 104°F in a standard, commercially available developer of the type suitable for use in a modern X-ray film processing machine having a total dry-to-dry process time of 90 seconds. The relative log speeds, fog levels, average contrast and

D-max were measured and the results are shown in Tables VI to X.

Table VI

| 5  | Compound added (Example No.) | Quantity added (mM/M) | Fog  | Relative log speed (0.5) | Average contrast | D-max |
|----|------------------------------|-----------------------|------|--------------------------|------------------|-------|
| 10 | No addition                  | —                     | 0.11 | 1.45                     | 0.55             | 1.28  |
| 15 | Azodicarbonamide             | 0.625                 | 0.07 | 1.45                     | 0.65             | 1.28  |
|    |                              | 0.025                 | 0.10 | 1.54                     | 0.71             | 1.38  |
|    |                              | 0.075                 | 0.09 | 1.45                     | 0.60             | 1.29  |
|    | 4                            | 0.25                  | 0.08 | 1.41                     | 0.66             | 1.29  |
|    |                              | 0.75                  | 0.07 | 1.29                     | 0.70             | 1.30  |
|    |                              | 2.50                  | 0.07 | 1.21                     | 0.80             | 1.33  |
| 20 |                              | 0.025                 | 0.10 | 1.50                     | 0.60             | 1.28  |
|    |                              | 0.075                 | 0.10 | 1.52                     | 0.50             | 1.26  |
|    | 3                            | 0.25                  | 0.08 | 1.41                     | 0.67             | 1.26  |
|    |                              | 0.75                  | 0.08 | 1.34                     | 0.82             | 1.32  |
|    |                              | 2.50                  | 0.07 | 1.20                     | 0.97             | 1.35  |
|    |                              | 0.025                 | 0.08 | 1.45                     | 0.65             | 1.28  |
| 25 |                              | 0.075                 | 0.09 | 1.46                     | 0.72             | 1.38  |
|    | 11                           | 0.25                  | 0.07 | 1.44                     | 0.90             | 1.40  |
|    |                              | 0.75                  | 0.07 | 1.21                     | 0.74             | 1.30  |
|    |                              | 2.50                  | 0.07 | 1.04                     | 0.80             | 1.25  |
|    |                              |                       |      |                          |                  |       |

Table VII

| 25 | Compound added (Example No.) | Quantity added (mM/M) | Fog  | Relative log speed (0.5) | Average contrast | D-max |
|----|------------------------------|-----------------------|------|--------------------------|------------------|-------|
|    | No addition                  | —                     | 0.10 | 1.53                     | 0.86             | 1.42  |
| 30 | Azodicarbonamide             | 0.625                 | 0.08 | 1.48                     | 0.50             | 1.26  |
|    |                              | 0.025                 | 0.10 | 1.44                     | 0.81             | 1.30  |
|    |                              | 0.075                 | 0.11 | 1.42                     | —                | 1.20  |
|    | 20                           | 0.25                  | 0.09 | 1.54                     | 0.80             | 1.34  |
|    |                              | 0.75                  | 0.08 | 1.48                     | 0.78             | 1.32  |
|    |                              | 2.50                  | 0.08 | 1.37                     | 0.75             | 1.34  |
| 35 |                              | 0.025                 | 0.09 | 1.55                     | 0.91             | 1.40  |
|    |                              | 0.075                 | 0.08 | 1.42                     | 0.65             | 1.28  |
|    | 23                           | 0.25                  | 0.08 | 1.42                     | 0.96             | 1.43  |
|    |                              | 0.75                  | 0.08 | 1.47                     | 0.65             | 1.32  |
|    |                              | 2.50                  | 0.08 | 1.28                     | 0.60             | 1.20  |
|    |                              |                       |      |                          |                  |       |

Table VIII

| 40 | Compound added (Example No.) | Quantity added (mM/M) | Fog  | Relative log speed (0.5) | Average contrast | D-max |
|----|------------------------------|-----------------------|------|--------------------------|------------------|-------|
|    | No addition                  | —                     | 0.14 | 1.80                     | 1.74             | 2.27  |
| 45 | Azodicarbonamide             | 0.625                 | 0.08 | 1.66                     | 1.61             | 1.84  |
|    |                              | 0.025                 | 0.08 | 1.70                     | 1.77             | 2.17  |
|    |                              | 0.075                 | 0.08 | 1.57                     | 1.71             | 2.02  |
|    | 21                           | 0.25                  | 0.08 | 1.40                     | 1.85             | 2.14  |
|    |                              | 0.75                  | 0.07 | 1.06                     | 1.75             | 1.71  |
|    |                              | 2.50                  | 0.08 | 0.69                     | 1.79             | 1.28  |
| 50 |                              | 0.025                 | 0.10 | 1.71                     | 1.69             | 2.04  |
|    |                              | 0.075                 | 0.08 | 1.75                     | 1.69             | 2.21  |
|    | 13                           | 0.25                  | 0.07 | 1.59                     | 1.63             | 1.75  |
|    |                              | 0.75                  | 0.07 | 1.42                     | 1.76             | 1.90  |
|    |                              | 2.50                  | 0.07 | 1.26                     | 1.57             | 1.70  |
|    |                              |                       |      |                          |                  |       |

Table IX

| 55 | Compound added (Example No.) | Quantity added (mM/M) | Fog  | Relative log speed (0.5) | Average contrast | D-max |
|----|------------------------------|-----------------------|------|--------------------------|------------------|-------|
|    | No addition                  | —                     | 0.13 | 1.71                     | 1.36             | 1.77  |
| 60 | Azodicarbonamide             | 0.625                 | 0.08 | 1.66                     | 1.40             | 1.68  |
|    |                              | 0.025                 | 0.10 | 1.84                     | 1.51             | 2.20  |
|    |                              | 0.075                 | 0.11 | 1.68                     | 1.56             | 1.93  |
|    | 10                           | 0.25                  | 0.10 | 1.70                     | 1.72             | 2.17  |
|    |                              | 0.75                  | 0.09 | 1.66                     | 1.74             | 2.15  |
|    |                              | 2.50                  | 0.07 | 1.45                     | 1.54             | 1.73  |

Table X—Continued

| Compound added (Example No.) | Quantity added (mM/M) | Fog  | Relative log speed (0.5) | Average contrast | D-max |
|------------------------------|-----------------------|------|--------------------------|------------------|-------|
| No addition                  | —                     | 0.08 | 1.80                     | 1.72             | 2.05  |
| 15 Azodicarbonamide          | 0.625                 | 0.05 | 1.73                     | 1.66             | 1.89  |
|                              | 0.025                 | 0.05 | 1.70                     | 1.59             | 1.92  |
|                              | 0.075                 | 0.06 | 1.67                     | 1.69             | 2.00  |
|                              | 0.25                  | 0.05 | 1.54                     | 1.81             | 1.98  |
|                              | 0.75                  | 0.04 | 1.35                     | 1.83             | 1.88  |
|                              | 2.50                  | 0.04 | 1.15                     | 1.69             | 1.70  |
|                              | 0.025                 | 0.06 | 1.69                     | 1.67             | 1.89  |
| 17                           | 0.075                 | 0.06 | 1.71                     | 1.65             | 1.93  |
|                              | 0.25                  | 0.05 | 1.60                     | 1.78             | 2.15  |
|                              | 0.75                  | 0.04 | 1.43                     | 1.77             | 1.83  |
|                              | 2.50                  | 0.05 | 1.28                     | 1.69             | 1.78  |
|                              | 0.025                 | 0.05 | 1.71                     | 1.68             | 2.06  |
|                              | 0.075                 | 0.04 | 1.68                     | 1.59             | 1.83  |
| 16                           | 0.25                  | 0.05 | 1.59                     | 1.71             | 1.94  |
|                              | 0.75                  | 0.05 | 1.46                     | 1.92             | 2.18  |
|                              | 2.50                  | 0.04 | 1.28                     | 1.83             | 1.72  |
|                              | 0.025                 | 0.08 | 1.73                     | 1.73             | 2.06  |
|                              | 0.075                 | 0.07 | 1.74                     | 1.87             | 2.33  |
| 12                           | 0.25                  | 0.08 | 1.61                     | 1.85             | 2.23  |
|                              | 0.75                  | 0.04 | 1.45                     | 1.95             | 1.99  |
|                              | 2.50                  | 0.03 | 1.26                     | 1.79             | 1.87  |
|                              | 0.025                 | 0.09 | 1.73                     | 1.73             | 2.09  |
|                              | 0.075                 | 0.06 | 1.65                     | 1.64             | 2.05  |
| 14                           | 0.25                  | 0.05 | 1.63                     | 1.73             | 2.13  |
|                              | 0.75                  | 0.05 | 1.51                     | 1.78             | 1.95  |
|                              | 2.50                  | 0.07 | 1.31                     | 1.77             | 2.07  |
|                              | 0.025                 | 0.06 | 1.76                     | 1.79             | 2.00  |
|                              | 0.075                 | 0.06 | 1.75                     | 1.77             | 2.08  |
| 22                           | 0.25                  | 0.06 | 1.76                     | 1.77             | 2.05  |
|                              | 0.75                  | 0.09 | 1.79                     | 1.79             | 2.22  |
|                              | 2.50                  | 0.05 | 1.78                     | 1.71             | 1.94  |
|                              | 0.025                 | 0.07 | 1.73                     | 1.87             | 2.32  |
|                              | 0.075                 | 0.07 | 1.70                     | 1.79             | 2.19  |
| 24                           | 0.25                  | 0.07 | 1.68                     | 1.80             | 2.17  |
|                              | 0.75                  | 0.07 | 1.62                     | 1.78             | 2.21  |
|                              | 2.50                  | 0.05 | 1.45                     | 1.94             | 2.07  |
|                              | 0.025                 | 0.07 | 1.74                     | 1.70             | 2.00  |
|                              | 0.075                 | 0.06 | 1.72                     | 1.80             | 2.16  |
| 18                           | 0.25                  | 0.05 | 1.73                     | 1.92             | 2.25  |

Table X—Continued

| Compound added (Example No.) | Quantity added (mM/M) | Fog  | Relative log speed (0.5) | Average contrast | D-max |
|------------------------------|-----------------------|------|--------------------------|------------------|-------|
| 5                            | —                     | 0.75 | 0.05                     | 1.68             | 2.07  |
|                              | 2.50                  | 0.04 | 1.55                     | 1.93             | 1.93  |
|                              | 0.025                 | 0.06 | 1.69                     | 1.51             | 1.89  |
|                              | 0.075                 | 0.05 | 1.63                     | 1.88             | 2.32  |
|                              | 0.25                  | 0.25 | 1.38                     | 1.86             | 2.16  |
|                              | 0.75                  | 0.05 | 1.03                     | 2.04             | 1.91  |
|                              | 2.50                  | 0.04 | 0.55                     | 1.63             | 1.36  |
| 10 25                        | —                     | 0.75 | 0.05                     | 1.68             | 2.17  |
|                              | 2.50                  | 0.04 | 1.55                     | 1.93             | 1.93  |
|                              | 0.025                 | 0.06 | 1.69                     | 1.51             | 1.89  |
|                              | 0.075                 | 0.05 | 1.63                     | 1.88             | 2.32  |
|                              | 0.25                  | 0.25 | 1.38                     | 1.86             | 2.16  |
|                              | 0.75                  | 0.05 | 1.03                     | 2.04             | 1.91  |
|                              | 2.50                  | 0.04 | 0.55                     | 1.63             | 1.36  |

As can be seen from the results, azocarbonamides added to a silver halide emulsion acted as anti-fogging agents but did not reduce the photographic speed to any marked extent as compared with emulsions to which no addition had been made. Also it can be seen that in general the addition of an azocarbonamide gave a reduction in fog of about the same level as that obtained by adding azodicarbonamide. Further, less azocarbonamide was often required to give comparable antifogging effects.

### EXAMPLE 33

In order to test the suitability of some of the azocarbonamides of the invention for use in emulsions as described in our copending U.S. patent application Ser. Nos. 243,463 and 244,276, Example 32 was repeated and in addition to measurement of the photographic properties of the emulsions immediately after their preparation, samples were subjected to advanced aging by incubation for 7 days at 125°F and 60% relative humidity. The results are shown in the following Tables XI and XII.

Table XI

| Compound added (Example No.) | Quantity added (mM/M) | Initial properties |                    |                  | After incubation |      |                    |                  |      |
|------------------------------|-----------------------|--------------------|--------------------|------------------|------------------|------|--------------------|------------------|------|
|                              |                       | Fog                | Relative log speed | Average contrast | Dmax             | Fog  | Relative log speed | Average contrast | Dmax |
| No addition                  | —                     | 0.10               | 1.55               | 1.78             | 2.15             | 0.04 | 1.48               | 0.99             | 1.47 |
| 7 Azodicarbonamide           | 0.625                 | 0.04               | 1.56               | 1.59             | 1.91             | 0.03 | 1.41               | 1.055            | 1.45 |
|                              | 0.025                 | 0.05               | 1.19               | 1.70             | 1.84             | 0.03 | 1.41               | 1.13             | 1.51 |
|                              | 0.075                 | 0.06               | 0.89               | 1.68             | 1.45             | 0.03 | 1.35               | 1.18             | 1.56 |
|                              | 0.25                  | 0.05               | 0.38               | —                | 0.64             | 0.02 | 1.19               | 1.08             | 1.39 |
|                              | 0.75                  | 0.07               | —                  | —                | 0.27             | 0.02 | 0.99               | 1.07             | 1.26 |
|                              | 2.50                  | 0.05               | —                  | —                | 0.18             | 0.03 | —                  | —                | 0.18 |
|                              | 0.025                 | 0.06               | 0.97               | 1.58             | 1.43             | 0.03 | 1.40               | 1.16             | 1.49 |
| 8                            | 0.075                 | 0.05               | 0.67               | 1.60             | 1.07             | 0.04 | 1.28               | 1.22             | 1.51 |
|                              | 0.25                  | 0.06               | —                  | —                | 0.52             | 0.03 | 1.13               | 1.11             | 1.37 |
|                              | 0.75                  | 0.06               | —                  | —                | 0.24             | 0.03 | 0.90               | 1.09             | 1.23 |
|                              | 2.50                  | 0.05               | —                  | —                | 0.17             | 0.02 | —                  | —                | 0.19 |

Table XII

| Compound added (Example No.) | Quantity added (mM/M) | Initial properties |                    |                  | After incubation |      |                    |                  |      |
|------------------------------|-----------------------|--------------------|--------------------|------------------|------------------|------|--------------------|------------------|------|
|                              |                       | Fog                | Relative log speed | Average contrast | Dmax             | Fog  | Relative log speed | Average contrast | Dmax |
| No addition                  | —                     | 0.15               | 1.67               | 1.54             | 1.13             | 0.24 | 1.69               | 1.09             | 1.70 |
|                              | 0.625                 | 0.06               | 1.65               | 1.52             | 1.96             | 0.07 | 1.69               | 1.19             | 1.63 |

Table XII -- Continued

| Com-<br>ound<br>added<br>(Example<br>No.) | Quantity<br>added<br>(mM/M) | Initial properties             |               |                               |      | After incubation |                               |                               |      |
|-------------------------------------------|-----------------------------|--------------------------------|---------------|-------------------------------|------|------------------|-------------------------------|-------------------------------|------|
|                                           |                             | Rela-<br>tive<br>log-<br>speed |               | Aver-<br>age<br>con-<br>trast | Dmax | Fog              | Rela-<br>tive<br>log<br>speed | Aver-<br>age<br>con-<br>trast | Dmax |
|                                           |                             | Fog                            | log-<br>speed | Dmax                          | Fog  | log<br>speed     | Dmax                          | Dmax                          |      |
| 19                                        | 0.25                        | 0.08                           | 1.66          | 1.58                          | 2.14 | 0.09             | 1.71                          | 1.22                          | 1.76 |
|                                           | 0.75                        | 0.04                           | 1.57          | 1.48                          | 2.08 | 0.04             | 1.68                          | 1.41                          | 1.84 |
|                                           | 2.5                         | 0.03                           | 1.40          | 1.52                          | 2.06 | 0.03             | 1.57                          | 1.47                          | 1.73 |
|                                           | 7.5                         | 0.03                           | 1.07          | 1.73                          | 2.23 | 0.03             | 1.31                          | 1.38                          | 1.67 |
|                                           | 25.0                        | 0.01                           | 0.64          | 1.35                          | 1.30 | 0.02             | 0.99                          | 1.37                          | 1.63 |
|                                           | 0.25                        | 0.05                           | 0.47          | 1.58                          | 1.23 | 0.05             | 1.40                          | 1.33                          | 1.69 |
| 9                                         | 0.75                        | 0.04                           | —             | —                             | 0.21 | 0.05             | 0.43                          | 1.58                          | 1.02 |
|                                           | 2.5                         | 0.03                           | —             | —                             | 0.15 | 0.02             | —                             | —                             | 0.34 |
|                                           | 7.5                         | 0.06                           | —             | —                             | 0.16 | 0.02             | —                             | —                             | 0.12 |
|                                           | 25.0                        | 0.33                           | —             | —                             | 0.48 | 0.14             | —                             | —                             | 0.23 |
| 30                                        | 0.25                        | 0.05                           | 1.24          | 1.64                          | 2.03 | 0.05             | 1.67                          | 1.33                          | 1.69 |
|                                           | 0.75                        | 0.06                           | 1.08          | 1.55                          | 1.92 | 0.05             | 1.62                          | 1.50                          | 1.83 |
|                                           | 2.5                         | 0.05                           | 0.72          | 1.55                          | 1.57 | 0.04             | 1.50                          | 1.38                          | 1.67 |
|                                           | 7.5                         | 0.05                           | 0.30          | —                             | 0.86 | 0.03             | 1.15                          | 1.23                          | 1.60 |
|                                           | 25.0                        | 0.05                           | —             | —                             | 0.32 | 0.03             | 0.59                          | 1.32                          | 1.27 |

As can be seen from these results, the azocarbonamides which had quaternary ammonium substituents strongly desensitized the emulsion initially and also kept the fog at a low level, but then decomposed during incubation so that the light sensitivity of the emulsions returned while the fog was still kept at very low levels. These compounds are therefore suitable oxidizing agents for use as described in our copending U.S. patent application Ser. Nos. 243,463 and 244,276.

I claim:

1. A silver halide photographic emulsion which has in fog inhibiting reactive association therewith at least a fog inhibiting amount of an azocarbonamide having one azo-carbonamide group.

2. The emulsion of claim 1 which has in fog inhibiting reactive association therewith an azocarbonamide of the formula



wherein Ar is an aromatic group and R is a carbonamide.

3. The emulsion of claim 2 wherein the azocarbonamide has an oxidation potential of -0.08 to +0.50.

4. The emulsion of claim 2 wherein the azocarbonamide is hydrolytically unstable.

5. The emulsion of claim 2 wherein a substituent on the nitrogen atom of the carbonamide group of the azo-

carbonamide contains at least one quaternary ammonium group.

6. The emulsion of claim 5 wherein the azocarbonamide has the formula



wherein X represents one or more negatively charged ions sufficient to give the azocarbonamide electrical neutrality.

7. The emulsion of claim 2 wherein the aromatic group of the azocarbonamide is a phenyl or a naphthyl group.

8. Photographic element comprising a silver halide photographic emulsion which contains therein or in a layer adjacent thereto a fog inhibiting amount of an azocarbonamide of the formula:



40 wherein Ar is an aromatic group and R is a carbonamide.

9. The emulsion of claim 1 wherein the azocarbonamide is present in an amount of at least 0.025 millimoles per mole of silver.

10. The element of claim 8 wherein the azocarbonamide is present in an amount of at least 0.025 millimoles per moles of silver.

\* \* \* \* \*

UNITED STATES PATENT OFFICE  
CERTIFICATE OF CORRECTION

PATENT NO. : 3,900,321

DATED : August 19, 1975

INVENTOR(S) : Alan N. Ferguson

It is certified that error appears in the above-identified patent and that said Letters Patent are hereby corrected as shown below:

Col. 22, Line 64, under "D max" in Table XII "1.13" should be  
--2.13--.

Col. 23, Line 46, Claim 5, "meulsion" should be --emulsion--.

Signed and Sealed this

*eleventh Day of November 1975*

[SEAL]

*Attest:*

**RUTH C. MASON**  
*Attesting Officer*

**C. MARSHALL DANN**  
*Commissioner of Patents and Trademarks*